

# United States Patent Office

3,194,734

Patented July 13, 1965

1

3,194,734

## PROCESSES AND COMPOSITIONS FOR DYEING HAIR AND SIMILAR FIBERS

John Robert Seemuller, Paris, Roger Charle, Soisy-sous-Montmorency, and Charles Pigerol, Saint-Ouen, France, assignors to Societe Anonyme dite: L'Oreal, Paris, France

No Drawing. Filed June 1, 1961, Ser. No. 126,749  
Claims priority, application France July 29, 1955, 8,544, Patent 1,133,594; June 3, 1960, 829,122, Patent 1,264,707

21 Claims. (Cl. 167—88)

This invention relates to a process and composition for tinting hair and other keratinous materials. More in particular, this invention refers to the use of dihydroxy-5,6-indole, and its derivatives in the preparation of certain dyeing compositions.

This invention is a continuation-in-part of U.S. application Serial No. 829,213, filed March 24, 1959 (now abandoned), which was a continuation-in-part of application Serial No. 599,893, filed July 25, 1956 (now abandoned).

This invention is also an improvement over U.S. Patent No. 2,934,296, which discloses a process for tinting hair and other keratinous materials, using dihydroxy-5,6-indole in an acid solution, which is applied to the hair and then oxidized in order to fix the dihydroxy-5,6-indole.

It has heretofore been known that dihydroxyphenylalanine ("dopa"), may be converted to a brown pigment by certain enzymes, such conversion taking place over a long period of time. This process is so slow that it is unsuitable for dyeing live human hair.

In the processes referred to above, whether carried out in one step or two, with a given concentration of dihydroxy-5,6-indole and a given concentration of an oxidizing agent, a deep color is obtained.

According to these processes, when it is desired to obtain a lighter shade, it is necessary to either reduce the quantity of the dihydroxy-5,6-indole while maintaining the same concentration of oxidizing agent, or keep the same concentration of dihydroxy-5,6-indole, and considerably increase the concentration of the oxidizing agent.

That is, the dihydroxy-5,6-indole normally produces a black or deep brown color, and when it is desired to obtain a lighter color, it is necessary to destroy by oxidation a portion of the pigments after they have been formed, thus lightening the color produced by the remainder of the pigments. This destruction, which has a bleaching effect, takes place simultaneously with the dyeing.

It is thus necessary, in order to obtain a light shade, to first dye the hair black, and then partially bleach it. This involves two disadvantages, a waste of the dihydroxy-5,6-indole supplied at the beginning, and uneven results which are difficult to predict by reason of the heterogeneity of living hair and the difference in its affinities for the dye which varies from one person to another.

Another disadvantage is the impossibility of knowing the exact moment at which the formation of pigments stops and the bleaching, that is to say, the partial destruction of the pigment starts.

According to the present invention a process for dyeing human hair and other keratinous fibers comprises applying thereto an aqueous alkaline composition containing dihydroxy-5,6-indole and ammonia, an ammonium salt or an amine, allowing the hair or other keratinous fiber to remain in contact with the said composition until the desired shade is obtained and then rinsing the hair free of such composition.

It has now been found that certain methyl derivatives of dihydroxy-5,6-indole when used in a concentration molecularly equivalent to that of dihydroxy-5,6-indole

2

and applied in the same manner, permit lighter shades to be obtained. The use of methyl derivatives of dihydroxy-5,6-indole thus has the advantage that the lighter shades obtained do not result from the partial destruction of pigments which have already been formed, but, from the methyl derivatives of the dihydroxy-5,6-indole which are used.

It is an object of the present invention to use dihydroxy-5,6-indole and ammonia or ammonium salts or amines in dyeing live human hair.

Another object of this invention is to produce a hair dye, which contains at least one ingredient having the following general formula:

15



20

in which R, R<sub>1</sub>, and R<sub>2</sub> designate either hydrogen or a methyl group, at least one of the three, R, R<sub>1</sub>, R<sub>2</sub>, radicals being other than hydrogen.

The compositions responding to the above general formula are:

25

methyl-1-dihydroxy-5,6-indole



30

methyl-2-dihydroxy-5,6-indole



35

methyl-3-dihydroxy-5,6-indole



40

dimethyl-1,2-dihydroxy-5,6-indole



45

dimethyl-2,3-dihydroxy-5,6-indole



50

dimethyl-1,3-dihydroxy-5,6-indole



55

trimethyl-1,2,3-dihydroxy-5,6-indole



60

65

70

In the composition according to the invention, the said methyl derivatives of dihydroxy-5,6-indole are prepared in an aqueous solution or in the form of a cream. The term "aqueous solution" herein designates any solution, the principal solvent of which is water. These solutions may comprise other solvents miscible in water, such as ethyl alcohol, isopropyl alcohol, glycols, esters of glycol, etc.

The invention also relates to a process for the dyeing of hair which is characterized by the fact that the hair is impregnated with a solution or a cream containing at least one derivative of dihydroxy-5,6-indole having the following formula:



in which R, R<sub>1</sub>, R<sub>2</sub> designate hydrogen or a methyl radical, at least one of the three radicals R, R<sub>1</sub> and R<sub>2</sub> being other than hydrogen, and in which the color is developed by an oxidizing agent.

The concentrations of the said methyl derivative of dihydroxy-5,6-indole, which are applied to the hair may vary within broad limits, but falls generally between 0.2% and 6% by weight of the solution and falls preferably between 0.5% and 3%.

Particularly suitable oxidizing agents include: hydrogen peroxide, sodium bromate, sodium percarbonate, sodium persulfate, ammonium persulfate, etc.

This invention is directed to a new hair dye and to hair dyed with this new dye.

The process according to the invention may be carried out in various ways.

One method is carried out in two steps. The hair is first impregnated within an aqueous solution of one of said methyl derivatives of dihydroxy-5,6-indole, the pH of this solution being less than or equal to 7. After a brief drying with a towel, for example, the color is then developed in situ by a second step consisting of the application of an aqueous solution containing an oxidizing reagent.

When the pH of the oxidizing solution is greater than 7 the following may be used as oxidizing reagents: hydrogen peroxide, sodium bromate, sodium percarbonate, sodium persulfate, ammonium persulfate, etc.

In this case, the oxidizing agent is added at the time of use to an aqueous solution of a nitrogen containing base, such as ammonia or an organic amine. Among the most suitable organic amines, are mono-, di-, and triethanolamine and the methyl, dimethyl and diethylamines. The concentration of the nitrogen containing base is preferably between 1% and 4% by weight of the total solution.

The ammonia or the organic bases may be used in the form of their salts, for example, as phosphates, carbonates, and bicarbonates.

When the pH of the oxidizing solution is less than 7, ammonium persulfate or sodium persulfate may be used.

In this case the persulfate selected may be added at the time of use to an aqueous solution of an organic acid, such as lactic acid or monochloroacetic acid. The concentration of the organic acid should preferably be between 1% and 10% by weight.

The quantities of oxidizing agents used, whether in alkaline or acid solutions, range preferably between 0.1% and 6% by weight of the total solution.

In the method of carrying out the invention, the second step may simply consist of oxidation by exposure to the air.

In the second single-step method of carrying out the invention, a solution containing one of the said methyl derivatives of dihydroxy-5,6-indole, is applied to the hair. This solution is at a pH equal to or greater than 7. This

solution, which is prepared, immediately before the application to the hair, results from the mixture of two solutions A and B, solution A containing a methylated derivative of dihydroxy-5,6-indole and solution B being an oxidizing solution.

Solution A is an aqueous solution containing as hereinbefore indicated, one of the methylated derivatives of dihydroxy-5,6-indole, the pH of this solution being adjusted to be equal to or greater than 7. The pH is adjusted by adding an alkaline agent, while taking care to exclude the air, by operating in a nitrogen atmosphere. However, the addition of this alkaline agent may also be carried out in the presence of air, if there is added an organic or mineral reducing agent which retards the oxidizing action of the oxygen in the air.

The alkaline agents which may be used to regulate the pH are: ammonia, its salts, such as triammonium phosphate, ammonium carbonate, ammonium bicarbonate, and a mixture of ammonium hydroxide and caustic soda, etc., organic amines such as monoethanolamine, diethanolamine, triethanolamine, methylamine, ethylamine, dimethylamine, diethylamine, etc.

The concentration of the alkaline agents, which is preferably between 1% and 15% by weight of the solution, is such that the pH is between 7 and 10.

When a mixture of ammonia or ammoniacal salts with caustic soda is used, the quantity of soda should not exceed 5% of the quantity of ammonia, that is to say, it should constitute no more than 0.75% by weight of the total solution.

The reducing agents which may be used to prevent the premature oxidation of the methyl derivative of dihydroxy-5,6-indole may be carboxylic mercaptans, such as thioglycolic acid, thiolactic acid, or mercapto alcohols, such as thioglycerol or even inorganic reducing agents, such as sodium sulfite. Their concentration may vary between 0.1% and 1% of the total solution.

It has also been established that it is also desirable to add to the solutions of methylated derivatives of dihydroxy-5,6-indole, a metal chelating or sequestering agent, such for instance, as the acid ethylenediamine-N-dihydroxyethyl-N'-diacetic acid of the formula:



the ethylenediamine tetraacetic acid having the formula:



the trisodium salt of N-hydroxyethyl-ethylenediamine triacetic acid, cyclohexane 1,2-diamine N, N' tetracetic acid having the formula:



A certain quantity of sodium chloride may advantageously be added to the aqueous solution of the methylated derivatives of hydroxy-5,6-indole. The addition of this salt produces certain shades of greater intensities for a given concentration of the indole derivatives.

The B solution is an aqueous solution containing an oxidizing agent and may be selected from the group comprising hydrogen peroxide, sodium bromate, sodium percarbonate, sodium persulfate, etc. The concentration of these oxidizing agents may vary from 0.2% to 12% of the oxidizing solution.

In order to apply the dyeing solution, the solution is mixed at the time of use, volume for volume; the solution A of a methylated derivative of dihydroxy-5,6-in-

dole and oxidizing agent B. The mixture is applied directly to the hair and left in contact with it for a variable time, not greater than an hour, the hair is rinsed, lightly shampooed to eliminate any excess dye, and dried.

Finally, the process according to the invention may be carried out, not only by means of aqueous solutions, but also by means of creams. In this case, the methylated derivatives of dihydroxy-5,6-indole are incorporated into a base consisting of a cream, which may have either an acid or alkaline pH. The hair may then be dyed in either one step or two.

When using the two-step process the hair is first impregnated with the cream at an acid pH. The cream is then removed by rinsing, and an oxidizing solution, similar to the solution B, hereinbefore described, applied to the hair.

When the hair is dyed in a single step, the cream containing the methylated derivative of dihydroxy-5,6-indole is mixed immediately before application with an oxidizing solution of the type B, hereinbefore described, and the mixture is then applied to the hair.

Of course, it is also possible to obtain intermediate shades by mixing several of the different methylated derivatives of dihydroxy-5,6-indole. In this case the sum of the weight of the methylated derivatives of dihydroxy-5,6-indole should not exceed 6% by weight of the solution.

When using dihydroxy-5,6-indole or its derivatives it is probable that the reaction proceeds through the formation of its orthoquinone derivatives, which are converted into pigments. It is thought that the pigments obtained are comparable to the natural melanic pigments existing in the hair, such as they are described in the literature (H. Weil-Malherbe, "The Constitution of Melanin," Annual Review of Biochemistry, vol. XVII—1948, pp. 7-8; Beer, Broadhurst and Robertson, "Chemistry of the Melanins"—Part V, Journal of the Chemical Society, 1954, pp. 1947-1953; Harold Burton, "Some Aspects of the Oxidative Dyeing of Keratinous Proteins," Soap, Perfumery and Cosmetics (London) August 1952, pages 834-836).

The invention will be better understood from the following examples, which are added by way of explanation and are not to limit the scope of the invention.

#### EXAMPLE 1

|                                                                                               |    |     |
|-----------------------------------------------------------------------------------------------|----|-----|
| 5,6-diacetoxindole                                                                            | gr | 1   |
| "Cemulsol 132" (a non-ionogen condensation product of ethylene oxide and a naphthol compound) | gr | 9   |
| Monoethanolamine                                                                              | gr | 2   |
| Thioglycolic acid (50%)                                                                       | gr | 0.1 |
| Water to make                                                                                 | cc | 100 |

This solution of 5,6-diacetoxindole was prepared in water with heating at about 50-60° C. until complete dissolution of the various ingredients. This temperature increase brings about the deacetylation and therefore the formation of the 5,6-hydroxyindole.

This solution is applied cool to the hair for 20 minutes, and the hair is then rinsed with water to remove the excess solution. White hair is dyed a light ash blond shade. The solution thus prepared comprises no accelerating agent and may be applied several times in succession, thus causing a progressive darkening of the shade obtained.

#### EXAMPLE 2

|                         |    |     |
|-------------------------|----|-----|
| 5,6-diacetoxindole      | gr | 1   |
| "Cemulsol 132"          | gr | 9   |
| Ammonia (20%)           | gr | 3   |
| Thioglycolic acid (50%) | gr | 0.1 |
| Water to make           | cc | 100 |

To 50 cc. of this solution there are added, immediately before use, 5 cc. of a 6 percent hydrogen peroxide solution, the mixture then being applied to the hair and al-

lowed to act on it for about 20 minutes. The hair is dyed a very fine metallic grey shade.

#### EXAMPLE 3

|    |                         |    |     |
|----|-------------------------|----|-----|
| 5  | 5,6-diacetoxindole      | gr | 1   |
|    | "Cemulsol 132"          | gr | 9   |
|    | Urea                    | gr | 7.5 |
|    | Diethylamine            | gr | 2   |
| 10 | Thioglycolic acid (50%) | gr | 0.1 |
|    | Water to make           | cc | 100 |

To 50 cc. of this solution there is added, immediately before use, 1 gr. of ammonium persulfate as an oxidizing agent. The solution is applied to the hair and allowed to act for 20 minutes. An ash blond coloring is obtained.

#### EXAMPLE 4

|    |                         |    |     |
|----|-------------------------|----|-----|
| 5  | 5,6-diacetoxindole      | gr | 1   |
|    | "Cemulsol 132"          | gr | 9   |
| 20 | Ammonia (20%)           | gr | 3   |
|    | Thioglycolic acid (50%) | gr | 0.1 |
|    | Water to make           | cc | 100 |

To 50 cc. of this solution there is added, immediately before use, 0.1 gr. of cobalt chloride as an oxidation catalyst. The solution is applied to the hair and allowed to act for 20 minutes. A bluish-grey shade is obtained.

#### EXAMPLE 5

|    |                         |    |     |
|----|-------------------------|----|-----|
| 5  | 5,6-diacetoxindole      | gr | 1   |
| 30 | "Cemulsol 132"          | gr | 9   |
|    | Ammonia (20%)           | gr | 3   |
|    | Trioglycolic acid (50%) | gr | 0.1 |
|    | Water to make           | cc | 100 |

To 50 cc. of this solution there is added at the time of use 0.1 gr. of manganese lactate (catalyst), whereafter the solution is applied to the hair, and allowed to act for 20 minutes. A bluish-grey shade is obtained.

#### EXAMPLE 6

|    |                         |    |     |
|----|-------------------------|----|-----|
| 40 | 5,6-diacetoxindole      | gr | 1   |
|    | Acetone                 | gr | 20  |
|    | Diethanolamine          | gr | 2   |
|    | Thioglycolic acid (50%) | gr | 0.1 |
|    | Water to make           | cc | 100 |

45 This solution is applied to the hair and allowed to act for 20 minutes. The hair is then rinsed and 50 cc. of a 1% cobalt chloride solution (serving as oxidation catalyst) is applied, and allowed to act for 5 minutes. The hair is rinsed and a very distinctive dark ash blond color is obtained.

#### EXAMPLE 7

|    |                         |    |     |
|----|-------------------------|----|-----|
| 5  | 5,6-diacetoxindole      | gr | 1   |
|    | "Cemulsol 132"          | gr | 9   |
|    | Ammonia (20%)           | gr | 3   |
| 55 | Thioglycolic acid (50%) | gr | 0.1 |
|    | Water to make           | cc | 100 |

50 cc. of this solution are applied to the hair and allowed to act for 15 minutes. At the end of this period the hair is rinsed and 50 cc. of an ammoniacal silver nitrate solution equivalent to a 0.1 percent silver oxide content is applied. A fine normal to dark chestnut shade is obtained.

#### EXAMPLE 8

|    |                         |    |     |
|----|-------------------------|----|-----|
| 65 | 5,6-diacetoxindole      | gr | 1   |
|    | "Cemulsol 132"          | gr | 9   |
|    | Monoethanolamine        | gr | 2   |
|    | Thioglycolic acid (50%) | gr | 0.1 |
|    | Water to make           | cc | 100 |

70 50 cc. of this solution are applied to the hair and allowed to act for 15 minutes. At the end of this period, the hair is rinsed and 50 cc. of an ammoniacal silver nitrate solution equivalent to 0.1 percent silver oxide content is applied. A fine reddish chestnut shade is obtained.

7  
EXAMPLE 9

|                         |           |
|-------------------------|-----------|
| 5,6-diacetoxindole      | gr. 1     |
| "Cemulsol 132"          | gr. 9     |
| Triammonium phosphate   | gr. 4     |
| Thioglycolic acid (50%) | gr. 0.1 5 |
| Water to make           | cc. 100   |

50 cc. of this solution are applied to the hair and allowed to act for 20 minutes. The hair is thereafter rinsed and an ammoniacal silver nitrate solution equivalent to a 0.25 percent silver oxide content is applied. A dark gold blond shade is obtained.

## EXAMPLE 10

|                         |         |
|-------------------------|---------|
| 5,6-diacetoxindole      | gr. 1   |
| "Cemulsol 132"          | gr. 9   |
| Ammonium carbonate      | gr. 4   |
| Thioglycolic acid (50%) | gr. 0.1 |
| Water to make           | cc. 100 |

50 cc. of this solution are applied to the hair and allowed to act for 20 minutes. The hair is thereafter rinsed and a silver nitrate solution equivalent to a 0.25 percent silver oxide content is applied. A gold blond shade is obtained.

In the foregoing Examples 1 to 10, the function of the thioglycolic acid is only to avoid a premature oxidation; thus it has a preservative function; the thioglycolic acid may be replaced by another reducing agent having the same protective function, such as e.g. thioglycerol, sodium sulfite.

## EXAMPLE 11

A cream product is prepared by emulsifying 20 parts of glycol stearate in 80 parts of a solution containing the 5,6 - diacetoxindole, monoethanolamine, thioglycolic acid and "Cemulsol 132," as described in Example 8. This cream is brushed on the hair and allowed to act for about 20 minutes. The hair is then rinsed and 50 cc. of an ammoniacal silver nitrate solution equivalent to a 0.1 percent silver oxide content are applied. A rather distinguished golden chestnut shade is obtained.

## EXAMPLE 12

A solution is prepared containing:

|                                                                              |         |
|------------------------------------------------------------------------------|---------|
| Methyl-2-dihydroxy-5,6-indole                                                | gr. 1   |
| Ammonia (20%)                                                                | gr. 8   |
| Thioglycolic acid                                                            | gr. 0.3 |
| Ethylenediamine N-dihydroxyethyl-N'-diacetic acid<br>(as sequestering agent) | grN 0.2 |
| Water to make                                                                | cc. 100 |

The pH of this solution is about 9.5.

The hair is impregnated with this solution, and after 10 to 30 minutes of impregnation the hair is rinsed. Then there is applied to the hair a solution containing, by weight:

|                                                                      |         |
|----------------------------------------------------------------------|---------|
| Hydrogen peroxide (20 volumes) (or 6% hydrogen<br>peroxide solution) | gr. 2.5 |
| Ammonia (20%)                                                        | gr. 14  |
| NaCl                                                                 | gr. 3.5 |
| Water to make                                                        | cc. 100 |

The hair is allowed to remain impregnated with this last solution during about 10 minutes. A reddish light brown shade is obtained.

The presence of sodium chloride is not indispensable in the second solution, but there is found that the results are improved thereby.

Instead of impregnating separately and successively the hair with the aforementioned first solution containing the methyl-2-dihydroxy-5,6-indole and with the recited second oxidizing solution containing hydrogen peroxide, with an intermediate rinsing, both solutions may be mixed together and the resulting solution may be applied immediately to the hair. However, in this second application process in one step, the hair is dyed a less intense shade.

8  
EXAMPLE 13

|                                                    |         |
|----------------------------------------------------|---------|
| On the one hand a solution is prepared containing: |         |
| Methyl-3-dihydroxy-5,6-indole                      | gr. 4   |
| Ammonia (20%)                                      | gr. 24  |
| Thioglycerol                                       | gr. 0.5 |
| Sequestering or complexing agent                   | gr. 0.2 |
| Water to make                                      | cc. 100 |

|                                                                      |         |
|----------------------------------------------------------------------|---------|
| On the other hand a solution is prepared containing:                 |         |
| Hydrogen peroxide (20 volumes) (or 6% hydrogen<br>peroxide solution) | gr. 50  |
| Water to make                                                        | cc. 100 |

These two solutions are mixed and the resulting mix is applied to white hair. After 15 to 40 minutes the hair is dyed black shade with violet glints.

## EXAMPLE 14

A solution is prepared containing:

|                                   |         |
|-----------------------------------|---------|
| Dimethyl-2,3-dihydroxy-5,6-indole | gr. 5   |
| Ammonia (20%)                     | gr. 24  |
| Sodium sulfite                    | gr. 0.2 |
| Sequestering agent                | gr. 0.2 |
| Water to make                     | cc. 100 |

Another solution is prepared containing:

|                                                                      |         |
|----------------------------------------------------------------------|---------|
| Hydrogen peroxide (20 volumes) (or 6% hydrogen<br>peroxide solution) | gr. 50  |
| Water to make                                                        | cc. 100 |

At the time of use equal volumes of the above-mentioned solutions are mixed. White hair impregnated with such mix is dyed more or less dark grey according to the duration of application (15 to 40 minutes) and the character of the hair.

## EXAMPLE 15

A solution is prepared containing:

|                                                         |         |
|---------------------------------------------------------|---------|
| Dimethyl-2,3-dihydroxy-5,6-indole                       | gr. 4   |
| Solution of methylamine (33%)                           | gr. 12  |
| Complexing or sequestering agent of the recited<br>type | gr. 0.2 |
| Water to make                                           | cc. 100 |

Before the use this solution is mixed with a 1:1 volume ratio with an oxidizing solution containing:

|                                                                      |         |
|----------------------------------------------------------------------|---------|
| Hydrogen peroxide (20 volumes) (or 6% hydrogen<br>peroxide solution) | gr. 40  |
| Water to make                                                        | cc. 100 |

Under the same application conditions as in the preceding example, white hair is dyed dark grey.

## EXAMPLE 16

A first solution is prepared containing:

|                               |         |
|-------------------------------|---------|
| Methyl-3-dihydroxy-5,6-indole | gr. 3   |
| Thioglycolic acid             | gr. 1   |
| Sequestering agent            | gr. 0.2 |
| Water to make                 | cc. 100 |

A second solution is prepared containing:

|                |         |
|----------------|---------|
| Sodium bromate | gr. 10  |
| Ammonia (20%)  | gr. 12  |
| Water to make  | cc. 100 |

Said both solutions are mixed in a volume ratio of 1:1, immediately before applying the mix to the hair to be tinted. White hair impregnated with this freshly prepared mix is dyed medium gray after a duration which does not practically exceed 40 minutes.

## EXAMPLE 17

A first solution is prepared containing:

|                                  |         |
|----------------------------------|---------|
| Methyl-2-dihydroxy-5,6-indole    | gr. 4   |
| Thiolactic acid                  | gr. 1   |
| Complexing or sequestering agent | gr. 0.2 |
| Water to make                    | cc. 100 |

A second solution is prepared containing:

|                     |     |     |
|---------------------|-----|-----|
| Sodium percarbonate | gr. | 8   |
| Ammonia (20%)       | gr. | 12  |
| Water to make       | cc. | 100 |

Immediately before the use equal volumes of these two solutions are mixed and hair to be dyed is impregnated with the resulting mix. White hair so impregnated is dyed dark blond shade within about 15 to 40 minutes.

#### EXAMPLE 18

A solution is prepared containing:

|                         |     |      |
|-------------------------|-----|------|
| Dihydroxy-5,6-indole    | gr. | 0.63 |
| "Cemulsol 132"          | gr. | 9    |
| Thioglycolic acid (80%) | gr. | 0.1  |
| Ammonia (20%)           | gr. | 3    |
| Water to make           | cc. | 100  |

To 50 cc. of this solution there are added, immediately before use, 5 cc. of a 6% hydrogen peroxide solution, the mixture then being applied to the hair and allowed to set on it for 20 minutes. The hair is dyed a very fine metallic grey shade.

#### EXAMPLE 19

In the two-step process using the methyl derivatives of dihydroxy-5,6-indole a solution is prepared having the following composition:

|                               |     |     |
|-------------------------------|-----|-----|
| Methyl-1-dihydroxy-5,6-indole | gr. | 1   |
| Acetic acid                   | cc. | 1   |
| Water to make                 | cc. | 100 |

This solution is applied to the hair and remains in contact therewith for about 20 minutes, then there is applied the following solution:

|                          |     |     |
|--------------------------|-----|-----|
| Ammonium hydroxide (20%) | cc. | 14  |
| Hydrogen peroxide (6%)   | cc. | 2.5 |
| Water to make            | cc. | 100 |

This is left in contact with the hair for 20 minutes, rinsed, shampooed and rinsed the second time and dried. A deep brown chestnut shade with a greenish glint is obtained.

#### EXAMPLE 20

A solution is prepared containing the following ingredients:

|                               |     |     |
|-------------------------------|-----|-----|
| Methyl-2-dihydroxy-5,6-indole | gr. | 1   |
| Acetic acid                   | cc. | 5   |
| Water to make                 | cc. | 100 |

This solution is applied to live grey hair, allowed to remain in contact therewith for 20 minutes, then there is applied a second solution having the same composition as the oxidizing solution called for in Example 19 and is applied in the same manner. A chestnut red shade is obtained.

#### EXAMPLE 21

A solution is prepared comprising:

|                               |     |     |
|-------------------------------|-----|-----|
| Methyl-3-dihydroxy-5,6-indole | gr. | 1.2 |
| Acetic acid                   | cc. | 3   |
| Water to make                 | cc. | 100 |

This solution is applied to grey hair, allowed to remain in contact therewith for 20 minutes, then there is applied the following solution:

|                          |     |     |
|--------------------------|-----|-----|
| Ammonium hydroxide (20%) | cc. | 12  |
| Hydrogen peroxide (6%)   | cc. | 4   |
| Water to make            | cc. | 100 |

This solution is allowed to remain in contact with the hair for 20 minutes, the hair is then rinsed, shampooed, rinsed the second time and dried. This hair is dyed a very deep violet shade.

#### EXAMPLE 22

The following solution is prepared:

|                                   |     |     |
|-----------------------------------|-----|-----|
| Dimethyl-1,2-dihydroxy-5,6-indole | gr. | 1.5 |
| Lactic acid                       | cc. | 5   |
| Butylglycol                       | cc. | 10  |
| Water to make                     | cc. | 100 |

This solution is applied to grey hair and allowed to remain in contact therewith for 20 minutes, then a second solution is applied, which contains:

|                          |     |     |
|--------------------------|-----|-----|
| Ammonium hydroxide (20%) | cc. | 8   |
| Hydrogen peroxide (6%)   | cc. | 10  |
| Water to make            | cc. | 100 |

This second solution is allowed to remain in contact with the hair for 20 minutes, it is then rinsed, shampooed, rinsed the second time and then dried. The hair has been dyed a clear ash blond.

#### EXAMPLE 23

The following solution is prepared:

|                                   |     |     |
|-----------------------------------|-----|-----|
| Dimethyl-2,3-dihydroxy-5,6-indole | gr. | 1   |
| Acetic acid                       | cc. | 5   |
| Butylglycol                       | cc. | 15  |
| Water to make                     | cc. | 100 |

This solution is applied to grey hair and allowed to remain in contact therewith for 20 minutes, then the following solution is applied thereto:

|                          |     |     |
|--------------------------|-----|-----|
| Ammonium hydroxide (20%) | cc. | 14  |
| Hydrogen peroxide (6%)   | cc. | 3   |
| Water to make            | cc. | 100 |

This solution is allowed to remain in contact with the hair for 20 minutes, then rinsed, shampooed, rinsed the second time and dried. The hair is tinted a deep golden blond.

#### EXAMPLE 24

The following solution is prepared:

|                                   |     |     |
|-----------------------------------|-----|-----|
| Dimethyl-1,3-dihydroxy-5,6-indole | gr. | 2   |
| Butylglycol                       | cc. | 10  |
| Monochloroacetic acid             | cc. | 7   |
| Water to make                     | cc. | 100 |

This solution is applied to grey hair and allowed to remain in contact therewith for 20 minutes. Then a second solution is applied thereto having the following composition:

|                        |     |     |
|------------------------|-----|-----|
| Ammonia (20%)          | cc. | 15  |
| Hydrogen peroxide (6%) | cc. | 5   |
| Water to make          | cc. | 100 |

This solution is left in contact with the hair for 20 minutes and is then rinsed, shampooed, rinsed the second time and dried. A clear ashy chestnut color is obtained.

#### EXAMPLE 25

The following solution is prepared:

|                                      |     |     |
|--------------------------------------|-----|-----|
| Trimethyl-1,2,3-dihydroxy-5,6-indole | gr. | 0.8 |
| Butylglycol                          | cc. | 15  |
| Acetic acid                          | cc. | 2   |
| Water to make                        | cc. | 100 |

This solution is applied to grey hair and allowed to remain in contact therewith for 20 minutes.

The following solution is then applied thereto:

|                          |     |     |
|--------------------------|-----|-----|
| Ammonium hydroxide (20%) | cc. | 7   |
| Hydrogen peroxide (6%)   | cc. | 15  |
| Water to make            | cc. | 100 |

This solution is allowed to remain in contact with the hair for 20 minutes. It is then rinsed, shampooed, rinsed the second time and dried. The hair is dyed a golden blond.

75

**11**  
**EXAMPLE 26**

The following solution is prepared:

|                                   |    |     |
|-----------------------------------|----|-----|
| Dimethyl-1,3-dihydroxy-5,6-indole | gr | 1   |
| Butylglycol                       | cc | 10  |
| Acetic acid                       | cc | 5   |
| Water to make                     | cc | 100 |

This solution is applied to white hair and allowed to remain in contact therewith for 20 minutes.

Then there is applied a second solution having the following composition:

|                     |    |     |
|---------------------|----|-----|
| Ammonia (20%)       | cc | 14  |
| Sodium percarbonate | gr | 0.8 |
| Water to make       | cc | 100 |

The second solution is allowed to remain in contact with the hair for 20 minutes. It is then rinsed, shampooed, rinsed the second time and dried. The hair is dyed an iron grey.

**EXAMPLE 27**

The following solution is prepared:

|                               |    |     |
|-------------------------------|----|-----|
| Methyl-2-dihydroxy-5,6-indole | gr | 1.3 |
| Butylglycol                   | cc | 10  |
| Acetic acid                   | cc | 2   |
| Water to make                 | cc | 100 |

This solution is applied to grey hair and allowed to remain in contact therewith for 30 minutes with partial drying, then there is applied a second solution having the following composition:

|                                           |    |     |
|-------------------------------------------|----|-----|
| Monomethylamine (33% solution)            | cc | 10  |
| "Cemulsol No. 132" (naphthol oxyethylene) | gr | 9   |
| Hydrogen peroxide (6%)                    | cc | 3   |
| Water to make                             | cc | 100 |

This solution is applied to remain in contact with the hair for 30 minutes, it is rinsed, shampooed, rinsed the second time and dried. A clear reddish chestnut color is obtained.

**EXAMPLE 28**

The following solution is prepared:

|                                   |    |     |
|-----------------------------------|----|-----|
| Dimethyl-2,3-dihydroxy-5,6-indole | gr | 1.4 |
| Butylglycol                       | cc | 12  |
| Lactic acid                       | cc | 3   |
| Water to make                     | cc | 100 |

This solution is applied to grey hair and allowed to remain in contact therewith for 20 minutes. The hair is then rinsed and a second solution is applied, comprising:

|                     |    |     |
|---------------------|----|-----|
| Monoethanolamine    | gr | 3   |
| Ammonium persulfate | gr | 0.5 |
| Urea                | gr | 7.5 |
| Water to make       | cc | 100 |

This solution is allowed to remain in contact with the hair for 20 minutes, then rinsed, shampooed, rinsed the second time and dried. A golden blond color is obtained.

**EXAMPLE 29**

The following solution is prepared:

|                                   |    |     |
|-----------------------------------|----|-----|
| Dimethyl-2,3-dihydroxy-5,6-indole | gr | 1   |
| Butylglycol                       | cc | 10  |
| Lactic acid                       | cc | 7   |
| Water to make                     | cc | 100 |

This solution is applied to live white hair, is allowed to remain in contact therewith for 30 minutes. The hair is allowed to partially dry and then there is applied thereto to the following solution:

|                                           |    |     |
|-------------------------------------------|----|-----|
| Diethylamine                              | gr | 4   |
| "Cemulsol No. 132" (naphthol oxyethylene) | gr | 10  |
| Sodium percarbonate                       | gr | 0.8 |
| Water to make                             | cc | 100 |

**12**

This solution is allowed to remain in contact with the hair for 30 minutes. The hair is then rinsed, shampooed, rinsed the second time and dried. The hair is tinted a clear golden blond.

**EXAMPLE 30**

The following solution is prepared:

|                               |    |     |
|-------------------------------|----|-----|
| Methyl-3-dihydroxy-5,6-indole | gr | 2   |
| Butylglycol                   | cc | 6   |
| Lactic acid                   | cc | 5   |
| Water to make                 | cc | 100 |

This solution is applied to white hair and allowed to remain in contact therewith for 30 minutes. It is then rinsed and the second solution is applied thereto, which comprises:

|                  |    |     |
|------------------|----|-----|
| Monoethanolamine | gr | 4   |
| Urea             | gr | 9   |
| Sodium bromate   | gr | 1   |
| Water to make    | cc | 100 |

This solution is allowed to remain in contact with the hair for 30 minutes. It is then rinsed, shampooed, rinsed the second time and dried. The hair is tinted a grey color.

**EXAMPLE 31**

The following solution is prepared:

|                                   |    |     |
|-----------------------------------|----|-----|
| Dimethyl-2,3-dihydroxy-5,6-indole | gr | 0.6 |
| Butylglycol                       | cc | 4   |
| Dichloracetic acid                | cc | 1.5 |
| Water to make                     | cc | 100 |

This solution is applied to live very white hair and allowed to remain in contact therewith for 30 minutes, and partially dried. Then there is applied a second solution comprising:

|                     |    |     |
|---------------------|----|-----|
| Ammonium persulfate | gr | 0.5 |
| Dichloracetic acid  | gr | 3   |
| Water to make       | cc | 100 |

This solution is allowed to remain in contact with the hair for 30 minutes. Then it is rinsed, washed, rinsed the second time and dried. The hair is dyed a clear violine.

**EXAMPLE 32**

The following solution is prepared:

|                               |    |     |
|-------------------------------|----|-----|
| Methyl-1-dihydroxy-5,6-indole | gr | 1.2 |
| Butylglycol                   | cc | 10  |
| Lactic acid                   | cc | 0.5 |
| Water to make                 | cc | 100 |

This solution is applied to white hair and allowed to remain in contact therewith for 30 minutes. It is then rinsed and a second solution applied thereto, comprising:

|                     |    |     |
|---------------------|----|-----|
| Ammonium persulfate | gr | 0.6 |
| Lactic acid         | cc | 5   |
| Water to make       | cc | 100 |

This solution is allowed to remain in contact with the hair for 30 minutes. It is rinsed, shampooed, rinsed the second time and dried. The hair is dyed a clear ash chestnut.

**EXAMPLE 33**

Solution A comprises:

|                               |    |     |
|-------------------------------|----|-----|
| Methyl-3-dihydroxy-5,6-indole | gr | 3   |
| Thioglycolic acid             | gr | 1   |
| Sequestering agent            | gr | 0.2 |
| Ammonium hydroxide (20%)      | gr | 12  |
| Water to make                 | cc | 100 |

Solution B comprises:

|                |    |     |
|----------------|----|-----|
| Sodium bromate | gr | 10  |
| Water to make  | cc | 100 |

These two solutions are mixed, volume per volume, immediately before application to the hair to be tinted.

13

White hair impregnated with these solutions is tinted a clear grey after about 40 minutes. The hair is washed, rinsed and dried.

## EXAMPLE 34

Solution A comprises:

|                               |    |     |
|-------------------------------|----|-----|
| Methyl-2-dihydroxy-5,6-indole | gr | 4   |
| Thioacetic acid               | gr | 1   |
| Ammonium hydroxide (20%)      | gr | 12  |
| Sequestering agent            | gr | 0.2 |
| Water to make                 | cc | 100 |

Solution B comprises:

|                     |    |     |
|---------------------|----|-----|
| Sodium percarbonate | gr | 0.8 |
| Water to make       | cc | 100 |

Immediately before using equal volumes of the two solutions are mixed. This mixture is applied to the hair to be tinted and the same allowed to remain in contact therewith for 15 to 40 minutes. The hair is rinsed, shampooed, rinsed a second time and dried. White hair is dyed a dark blond.

## EXAMPLE 35

Solution A comprises:

|                               |    |     |
|-------------------------------|----|-----|
| Methyl-3-dihydroxy-5,6-indole | gr | 2   |
| Butylglycol                   | gr | 30  |
| Thioglycolic acid             | gr | 1   |
| Ammonium hydroxide (20%)      | gr | 20  |
| Sodium chloride               | gr | 6   |
| Sequestering agent            | gr | 0.3 |
| Water to make                 | cc | 100 |

Solution B comprises:

|                        |    |     |
|------------------------|----|-----|
| Hydrogen peroxide (6%) | gr | 50  |
| Water to make          | cc | 100 |

Solutions A and B are mixed at the time of their application to the hair. This mixture is applied to white or a clear blond hair and is allowed to remain in contact therewith for 20 minutes. The hair is rinsed, washed, rinsed again and dried. A violine color is obtained.

## EXAMPLE 36

Solution A comprises:

|                               |    |     |
|-------------------------------|----|-----|
| Methyl-3-dihydroxy-5,6-indole | gr | 3   |
| Butylglycol                   | gr | 30  |
| Thioglycolic acid             | gr | 1   |
| Sodium chloride               | gr | 6   |
| Sequestering agent            | gr | 0.3 |
| Ammonium carbonate            | gr | 10  |
| Water to make                 | cc | 100 |

Solution B comprises:

|                        |    |     |
|------------------------|----|-----|
| Hydrogen peroxide (6%) | gr | 50  |
| Water to make          | cc | 100 |

Solutions A and B are mixed in equal volumes at the time of use. This mixture is applied to white hair and allowed to remain in contact therewith for 20 to 30 minutes. The hair is then rinsed, shampooed, rinsed the second time and dried. An intermediate violet color is obtained.

## EXAMPLE 37

Solution A comprises:

|                                   |    |     |
|-----------------------------------|----|-----|
| Dimethyl-2,3-dihydroxy-5,6-indole | gr | 4   |
| Butylglycol                       | gr | 20  |
| Thioglycolic acid                 | gr | 1   |
| Ammonium hydroxide (20%)          | gr | 20  |
| Sodium hydroxide                  | gr | 7   |
| Sodium chloride                   | gr | 6   |
| Sequestering agent                | gr | 0.3 |
| Water to make                     | cc | 100 |

Solution B comprises:

|                        |    |     |
|------------------------|----|-----|
| Hydrogen peroxide (6%) | gr | 40  |
| Water to make          | cc | 100 |

14

Solutions A and B are mixed in equal volumes and then applied to white hair and allowed to remain in contact therewith for 30 minutes. The hair is then rinsed, shampooed, rinsed the second time and dried. A strong blue-grey color is obtained.

## EXAMPLE 38

Solution A comprises:

|                               |    |     |
|-------------------------------|----|-----|
| Methyl-2-dihydroxy-5,6-indole | gr | 6   |
| Butylglycol                   | gr | 30  |
| Thioglycolic acid             | gr | 1   |
| Monoethanolamine              | gr | 16  |
| Sodium chloride               | gr | 4   |
| Sequestering agent            | gr | 0.3 |
| Water to make                 | cc | 100 |

Solution B comprises:

|                        |    |     |
|------------------------|----|-----|
| Hydrogen peroxide (6%) | gr | 60  |
| Water to make          | cc | 100 |

At the time of use equal volumes of Solutions A and B are mixed and then applied to white hair and allowed to remain in contact therewith for 20 minutes. The hair is then rinsed, shampooed, rinsed the second time and dried. A chestnut red color is obtained.

## EXAMPLE 39

Solution A comprises:

|                               |    |     |
|-------------------------------|----|-----|
| Methyl-1-dihydroxy-5,6-indole | gr | 4   |
| Butylglycol                   | gr | 30  |
| Thioglycolic acid             | gr | 1   |
| Ammonium hydroxide (20%)      | gr | 24  |
| Sodium chloride               | gr | 6   |
| Sequestering agent            | gr | 0.4 |
| Water to make                 | cc | 100 |

Solution B comprises:

|                        |    |     |
|------------------------|----|-----|
| Hydrogen peroxide (6%) | gr | 30  |
| Water to make          | cc | 100 |

Equal volumes of Solutions A and B are mixed at the time of use. This mixture is then applied to grey hair and allowed to remain in contact therewith for 20 to 30 minutes. The hair is then rinsed, shampooed, rinsed the second time and dried. A very clear chestnut with a green glint is obtained.

## EXAMPLE 40

Solution A comprises:

|                                   |    |     |
|-----------------------------------|----|-----|
| Dimethyl-1,2-dihydroxy-5,6-indole | gr | 4   |
| Butylglycol                       | gr | 20  |
| Thioglycolic acid                 | gr | 1   |
| Ammonium hydroxide (20%)          | gr | 24  |
| Sodium chloride                   | gr | 6   |
| Sequestering agent                | gr | 0.4 |
| Water to make                     | cc | 100 |

Solution B comprises:

|                        |    |     |
|------------------------|----|-----|
| Hydrogen peroxide (6%) | gr | 30  |
| Water to make          | cc | 100 |

Equal volumes of Solutions A and B are mixed at the time of application. This mixture is applied to white hair and allowed to remain in contact therewith for 20 to 30 minutes. The hair is then rinsed, shampooed, rinsed the second time and dried. A golden blond color is obtained.

## EXAMPLE 41

Solution A comprises:

|                                   |    |     |
|-----------------------------------|----|-----|
| Dimethyl-1,3-dihydroxy-5,6-indole | gr | 6   |
| Butylglycol                       | gr | 30  |
| Thioglycolic acid                 | gr | 1   |
| Ammonium hydroxide (20%)          | gr | 24  |
| Sodium chloride                   | gr | 6   |
| Sequestering agent                | gr | 0.4 |
| Water to make                     | cc | 100 |

## Solution B comprises:

|                        |         |
|------------------------|---------|
| Hydrogen peroxide (6%) | gr. 30  |
| Water to make          | cc. 100 |

Equal volumes of the two solutions are mixed at the time they are to be used. This mixture is applied to white hair and allowed to remain in contact therewith for 20 to 30 minutes. The hair is rinsed, shampooed, rinsed the second time and dried. A blond color is obtained.

## EXAMPLE 42

## Solution A comprises:

|                                      |         |
|--------------------------------------|---------|
| Trimethyl-1,2,3-dihydroxy-5,6-indole | gr. 6   |
| Butylglycol                          | gr. 30  |
| Thioglycolic acid                    | gr. 1   |
| Ammonium hydroxide (20%)             | gr. 24  |
| Sodium chloride                      | gr. 6   |
| Sequestering agent                   | gr. 0.4 |
| Water to make                        | cc. 100 |

## Solution B comprises:

|                        |         |
|------------------------|---------|
| Hydrogen peroxide (6%) | gr. 30  |
| Water to make          | cc. 100 |

Equal volumes of the two solutions are mixed just prior to use. The mixture is then applied to white hair and allowed to remain in contact therewith for 20 to 30 minutes. The hair is rinsed, shampooed, rinsed the second time and dried. A strong blond color is obtained.

## The application in the form of a cream

## EXAMPLE 43

## An acid tinctorial cream is prepared, which comprises:

|                                   |         |
|-----------------------------------|---------|
| Coconut fatty acid amides         | gr. 15  |
| Beeswax                           | gr. 5   |
| Dimethyl-2,3-dihydroxy-5,6-indole | gr. 1   |
| Acetic acid                       | gr. 1   |
| Water to make                     | cc. 100 |

The amide and the beeswax are thoroughly mixed and then there is introduced a solution of dimethyl-2,3-dihydroxy-5,6-indole dissolved in hot water and the acetic acid. This cream, after cooling is applied directly on the hair to be tinted and maintained in contact therewith for 20 minutes. The hair is then rinsed. It is dried with a towel and then a second solution is applied. This solution comprises:

|                          |         |
|--------------------------|---------|
| Ammonium hydroxide (20%) | gr. 14  |
| Hydrogen peroxide (6%)   | gr. 2.5 |
| Water to make            | cc. 100 |

The second solution is allowed to remain in contact with the hair for 20 minutes. The hair is rinsed, shampooed, rinsed again and dried. The hair is tinted a blond color.

## EXAMPLE 44

## An acid cream is prepared as in the preceding example which comprises:

|                               |         |
|-------------------------------|---------|
| Coconut fatty acid amides     | gr. 15  |
| Beeswax                       | gr. 5   |
| Methyl-1-dihydroxy-5,6-indole | gr. 0.5 |
| Methyl-2-dihydroxy-5,6-indole | gr. 0.5 |
| Acetic acid                   | gr. 1   |
| Water to make                 | cc. 100 |

This cream is applied to the hair for 20 minutes on white hair. It is then rinsed, dried with a towel and a second oxidizing solution as in the preceding example is then applied. This is allowed to remain in contact with the hair for 20 minutes. After rinsing, shampooing, and re-rinsing the hair is dried. A clear chestnut shade is obtained.

## EXAMPLE 45

An alkaline cream is prepared, comprising:

|                                   |         |
|-----------------------------------|---------|
| Coconut fatty acid amides         | gr. 30  |
| Beeswax                           | gr. 10  |
| Ammonium laurylsulfate            | gr. 8   |
| Methyl-2-dihydroxy-5,6-indole     | gr. 2   |
| Dimethyl-2,3-dihydroxy-5,6-indole | gr. 3   |
| Thioglycolic acid                 | gr. 1   |
| Butylglycol                       | gr. 6   |
| Ammonium hydroxide (20%)          | gr. 24  |
| Sodium chloride                   | gr. 4   |
| Sequestering agent                | gr. 0.4 |
| Water to make                     | cc. 100 |

An oxidizing solution is also prepared which comprises:

|                        |         |
|------------------------|---------|
| Hydrogen peroxide (9%) | gr. 60  |
| Water to make          | cc. 100 |

At the time of use equal parts of the alkaline cream and the oxidizing solution are mixed so as to obtain a homogeneous mixture. This is then applied to grey hair and allowed to remain in contact therewith for 20 to 30 minutes. The hair is then rinsed, shampooed, rinsed a second time and dried. The hair is dyed a blond rose.

What is claimed is:

1. A process for dyeing human hair which comprises applying thereto an aqueous alkaline composition containing a compound represented by the formula



in which R, R<sub>1</sub> and R<sub>2</sub> are selected from the group consisting of H and CH<sub>3</sub>, at least one of these radicals being CH<sub>3</sub>; and a nitrogenous substance selected from the group consisting of ammonia, ammonium salts and amines; and applying thereto in a second step an aqueous solution of a water soluble synthetic inorganic oxidizing agent; and allowing said composition to remain in contact with said hair until the desired shade is obtained.

2. A process for dyeing human hair which comprises saturating the fibrous material with an aqueous alkaline composition containing dihydroxy-5,6-indole and a nitrogenous substance selected from the group consisting of ammonia, ammonium salts and amines; and a sufficient amount of a water soluble synthetic inorganic oxidizing agent; and allowing said composition to remain in contact with said hair until a desired shade is obtained.

3. A process for dyeing human hair which comprises applying thereto in a first step an aqueous alkaline composition containing a compound represented by the formula



in which R, R<sub>1</sub> and R<sub>2</sub> are selected from the group consisting of H and CH<sub>3</sub>, at least one of these radicals being CH<sub>3</sub>; and a nitrogenous substance selected from the group consisting of ammonia, ammonium salts and amines; rinsing said hair and applying thereto in a second step an ammoniacal silver nitrate solution.

4. A process for dyeing human hair which comprises saturating in a first step the fibrous material with an aqueous alkaline composition containing dihydroxy-5,6-indole and a nitrogenous substance selected from the group consisting of ammonia, ammonium salts and amines; rinsing said fibrous material; and applying thereto in a second step an alkaline solution of a synthetic inorganic oxidizing agent.

5. A process according to claim 1 for dyeing human hair in which the oxidizing agent is added at the time of use to the oxidative dye substance.

6. A process according to claim 1 for dyeing human hair in which the oxidizing agent is applied to the hair after the hair has been impregnated with the oxidative dye substance.

7. A process according to claim 1 for dyeing human hair in which the oxidative dye substance is methyl-1 dihydroxy-5,6-indole.

8. A process according to claim 1 for dyeing human hair in which the oxidative dye substance is methyl-2 dihydroxy-5,6-indole.

9. A process according to claim 1 for dyeing human hair in which the oxidative dye substance is methyl-3 dihydroxy-5,6-indole.

10. A process according to claim 1 for dyeing human hair in which the oxidative dye substance is dimethyl-1,2 dihydroxy-5,6-indole.

11. A process according to claim 1 for dyeing human hair in which the oxidative dye substance is dimethyl-1,3 dihydroxy-5,6-indole.

12. A process according to claim 1 for dyeing human hair in which the oxidative dye substance is dimethyl-1,2,3 dihydroxy-5,6-indole.

13. A process according to claim 1 for dyeing human hair in which the oxidative dye substance is trimethyl-1,2,3 dihydroxy-5,6-indole.

14. A product suitable for dyeing live human hair by an oxidative process which comprises a water soluble solution of dihydroxy-5,6-indole having the formula



in which R, R<sub>1</sub> and R<sub>2</sub> are selected from the group consisting of H and CH<sub>3</sub>, at least one of these radicals being

30

2,539,202 1/51 Peck \_\_\_\_\_ 167-88 X

## OTHER REFERENCES

- Beer et al., J. of Chem. Soc., 1954, pp. 1947-1953.  
 Burton, J. S., Dyers and Colorists, vol. 66, September 1950, pp. 474-8.  
 35 Moncrieff, Manufacturing Chemist, 21:8, August 1950, pp. 330-4.

JULIAN S. LEVITT, Primary Examiner.

MORRIS O. WOLK, Examiner.

CH<sub>3</sub>, and the pH value of said solution being at least 7; and a nitrogenous substance selected from the group consisting of ammonia, ammonium salts and amines; and a sufficient amount of a water soluble oxidizing agent.

5 15. A product as claimed in claim 14 suitable for dyeing live human hair, in which the oxidative dye substance is methyl-1 dihydroxy-5,6-indole.

16. A product as claimed in claim 14 suitable for dyeing live human hair in which the oxidative dye substance is methyl-2 dihydroxy-5,6-indole.

10 17. A product as claimed in claim 14 suitable for dyeing live human hair in which the oxidative dye substance is methyl-3 dihydroxy-5,6-indole.

18. A product as claimed in claim 14 suitable for dyeing live human hair in which the oxidative dye substance is dimethyl-1,3 dihydroxy-5,6-indole.

19. A product as claimed in claim 14 suitable for dyeing live human hair in which the oxidative dye substance is dimethyl-1,3 dihydroxy-5,6-indole.

20. A product as claimed in claim 14 suitable for dyeing live human hair in which the oxidative dye substance is dimethyl-1,2,3 dihydroxy-5,6-indole.

21. A product as claimed in claim 14 suitable for dyeing live human hair in which the oxidative dye substance is trimethyl-1,2,3 dihydroxy-5,6-indole.

## References Cited by the Examiner

## UNITED STATES PATENTS

2,539,202 1/51 Peck \_\_\_\_\_ 167-88 X